

# United States Patent Office

2,724,633

Patented Nov. 22, 1955

1

2,724,633

## PROCESS OF MAKING CELLULOSE FIBERS CONTAINING ETHER GROUPS AND BETA-PROPIOLACTONE SUBSTITUENTS

George C. Daul, Robert M. Reinhardt, and John D. Reid, New Orleans, La., assignors to the United States of America as represented by the Secretary of Agriculture

No Drawing. Application May 14, 1954,  
Serial No. 430,001

8 Claims. (Cl. 8—120)

(Granted under Title 35, U. S. Code (1952), sec. 266)

A non-exclusive, irrevocable, royalty-free license in the invention herein described, for all governmental purposes, throughout the world, with the power to grant sublicenses for such purposes, is hereby granted to the Government of the United States of America.

This invention relates to a process of chemically modifying cellulose fibers. The invention provides fibers composed essentially of cellulose ethers and beta-propiolactone reaction products combined with cellulose, and provides an improved process of modifying cellulose fibers by reaction with beta-propiolactone.

This application is a continuation-in-part of our copending applications, Serial Nos. 299,772 and 393,523 filed July 18, 1952, and November 20, 1953.

Our copending application No. 299,772 relates to reacting cellulose fibers with beta-propiolactone at a temperature of from about 50 to 155° C. until fibers are produced containing from about 0.5 to 26%, based on the weight of the original cellulose fibers, of beta-propiolactone reaction products combined with the cellulose, i. e., about from 0.5 to 26% beta-propiolactone substituents. The substituted fibers so produced have markedly increased effective diameters, decreased affinity for water and polar compounds, and have a tensile strength not materially less than that of the fibers from which they are produced. They have a dye resistance, heat resistance, acid induced degradation resistance, wrinkle resistance, and wool-like properties markedly greater than those of the fibers from which they are produced. And, where desired, they can be converted to fibers containing an appreciable proportion of olefinic unsaturated groups.

A primary object of the present invention is to provide chemically modified cellulose fibers containing beta-propiolactone reaction products combined with the cellulose, which fibers have a heat resistance and acid degradation resistance greater than those of the fibers containing beta-propiolactone reaction products combined with cellulose heretofore known. A further object is to provide a process of producing fibers containing beta-propiolactone reaction products combined with cellulose, in which process the fibers exhibit an enhanced reactivity towards the beta-propiolactone. A further object is to provide chemically modified cellulose fibers containing beta-propiolactone reaction products combined with cellulose, in which fibers the somewhat wool-like properties of cellulose fibers containing beta-propiolactone reaction products combined with cellulose are modified by properties such as the altered dyestuff susceptibility, affinity for water (mold resistance, and the like) which are imparted to cellulose fibers by an etherification yielding a cellulose ether containing polar alkyl radicals.

In general, according to this invention, cellulose fibers containing ether groups and beta-propiolactone reaction products combined with cellulose are produced by etherifying cellulose fibers with an etherifying agent selected from the group consisting of aminoalkyl sulfuric acid wherein the aminoalkyl radical is the etherifying radical,

2

2-aminoethyl sulfuric acid being preferred, monochloroacetic acid wherein the carboxyalkyl and alkali metal carboxyalkyl radicals are the etherifying radicals, alkylene oxide wherein the hydroxylalkyl radical is the etherifying radical, ethylene oxide being preferred, acrylonitrile wherein the cyanoalkyl radical is the etherifying radical, and alkyl sulfate wherein the alkyl group is the etherifying radical, dimethyl sulfate being preferred, the alkyl group in each of said etherifying radicals having from 1 to 3 carbon atoms, until etherified cellulose fibers containing from about 0.1 to 2.5 of the said etherifying radicals of said etherifying agent per anhydroglucose unit is produced, and reacting the said etherified cellulose fibers with beta-propiolactone at a temperature of from 0° C. to a temperature slightly below the decomposition temperature of the fibers until fibers are produced containing from about 0.5 to 26%, based on the weight of the etherified fibers, of beta-propiolactone reaction products combined with the cellulose. Such fibers are composed of cellulose ethers containing, per each anhydroglucose unit, from about 0.1 to 2.5 radicals selected from the group consisting of aminoalkyl, alkali metal carboxyalkyl, carboxyalkyl, hydroxylalkyl, cyanoalkyl, and alkyl radicals, the alkyl group in each of said radicals having from 1 to 3 carbon atoms, and containing from about 0.5 to 26%, based on the weight of the cellulose ethers, of beta-propiolactone reaction products combined with cellulose.

When the etherified cellulose fibers are reacted with beta-propiolactone, their increased weight is essentially due to the introduction of beta-propiolactone reaction products within the walls of the fibers. This is true whether the etherified fibers are reacted with vapors of beta-propiolactone, or with beta-propiolactone in a liquid solution, in the presence or absence of a solvent or a catalyst, or in the presence of an acidic or a basic catalyst.

Cellulose fibers which can be used include cotton fibers such as lint, linters, and the like, and regenerated cellulose fibers such as viscose rayon fibers, before or after bleaching, mercerization, and the like treatments. Cotton fibers are preferred.

The cellulose fibers can be reacted in the form of free fibers, sliver, yarn, or fabric. The use of yarns, threads or cloth is preferred.

The etherification can be conducted in a variety of ways. For example, an etherification yielding ethers containing aminoalkyl radicals can be accomplished by reacting cellulose fibers with an aminoalkyl sulfuric acid in the presence of aqueous alkali metal hydroxide, by a process such as that described in U. S. Patent No. 2,459,222; one yielding ethers containing alkali metal carboxyalkyl radicals, or carboxyalkyl radicals, by reacting the fibers with monochloroacetic acid, by a process such as those of U. S. Patents Nos. 2,448,153, 2,617,707, or 2,663,615, and neutralizing the ether salt to yield the ether acid, where desired; one yielding ethers containing hydroxylalkyl radicals, by reacting the fibers with an alkylene oxide in the presence of aqueous alkali metal hydroxide, by a process such as is described in J. Soc. of Dyers and Colourists, volume 56, pp. 6-17, January 1940; one yielding cyanoalkyl radicals, by reacting the fibers with acrylonitrile in the presence of aqueous alkali metal hydroxide, by a process such as those described in U. S. Patent No. 2,375,848 or 2,473,308; and one yielding alkyl radicals, by reacting the fibers with an alkyl sulfate in the presence of aqueous alkali metal hydroxide, by a process such as is described in Textile Research Journal, volume 19, pp. 771-783, December 1949.

The etherification, particularly when the cellulose fibers are cotton fibers, is preferably one yielding ethers containing from about 0.1 to 1.0 aminoethyl or alkali metal

carboxymethyl radicals in which cotton fibers are reacted with ethyl sulfuric acid or monochloroacetic acid in the presence of aqueous sodium hydroxide.

The etherified fibers can be reacted with beta-propiolactone, solutions containing beta-propiolactone, or the vapors of beta-propiolactone or beta-propiolactone containing solutions. The fibers are preferably reacted by immersing them in a beta-propiolactone containing liquid maintained at from about 0° C. to a temperature slightly below the decomposition temperature of the etherified fibers. The beta-propiolactone containing liquid can be liquid beta-propiolactone or a solution of beta-propiolactone. The reaction is preferably continued until the fibers contain from about 0.5 to 26%, based on the weight of the etherified fibers, of beta-propiolactone reaction products combined with cellulose.

Suitable solvents for such solutions comprise liquids which are unreactive solvents for beta-propiolactone (i. e., are unreactive toward beta-propiolactone or cellulose and are capable of dissolving at least about 0.5 part of beta-propiolactone per part of solvent).

Throughout the specification and claims the term "parts" refers to parts by weight.

Examples of suitable solvents include hydrocarbons such as benzene, xylene, and the normal, branch-chain, or cyclic hexanes, halohydrocarbons such as carbon tetrachloride, chloroform, tetrachloroethane, and chlorobenzene, and ketones such as acetone, methyl iso-butyl ketone, and methyl iso-propyl ketone, and ethers such as dioxane and the like organic solvents. The use of solutions of beta-propiolactone containing from about 5 to 20 parts of solvent per part of beta-propiolactone and the use of amounts of such solutions providing from about 1 to 4 parts of beta-propiolactone per part of cellulose is preferred.

Preferred solvents comprise water miscible solvents such as water; liquid ketones such as acetone; liquid ethers such as dioxane; and the like. Where a solvent is employed the etherification reaction is preferably conducted by immersing the etherified cellulose fiber in the solvent solution maintained at the reaction temperature desired.

The reactivity of the etherified fibers towards beta-propiolactone is appreciably improved by the presence of a relatively small amount of water in intimate contact with the fibers. The amount of water can be varied widely, but, in general, the amount left in wetted fibers by the mechanical removal of excess moisture, using textile apparatus such as squeeze rolls or centrifuges, is particularly suitable. In a preferred embodiment of this invention, cellulose fibers are etherified, then wetted and mechanically freed of excess liquid, and the moist fibers are reacted with beta-propiolactone at a temperature of from about 5° to 150° C.

The reactivity of the etherified fibers is further improved when the water in contact with the fibers contains dissolved alkali metal hydroxide. The use of alkali metal hydroxide concentrations of from about 5 to 50% and the methods of pretreating the fibers with such a water solution which are more fully described in our copending application No. 393,523 comprise another preferred embodiment of the present invention.

Beta-propiolactone is known to be capable of reacting in numerous ways. For example, it can etherify hydroxyl groups, esterify hydroxyl groups, etherify carboxy groups, react with amino groups, and polymerize. Presumably, the beta-propiolactone undergoes a plurality of types of reactions when it is reacted with the etherified cellulose fibers in accordance with this invention.

Following the beta-propiolactone reaction, the fibers are preferably washed free of uncombined reactants with an organic solvent capable of dissolving polymers of beta-propiolactone, for example, with solvents such as acetone, alcohol, or dioxane. The washing substantially completely removes adhering beta-propiolactone polymeric

products which are not chemically attached to the fiber walls, and leaves the fibers with a soft, wool-like hand and feel.

When cotton fibers are: (1) etherified to yield cellulose ethers containing from about 0.1 to 1 ether radical per anhydroglucose unit under mild conditions that preserve the bulk of the performance characteristics inherent in the intricate structure of the fibers; (2) then are reacted with beta-propiolactone at a temperature below about 150° C.; the etherification and the beta-propiolactone reactions coact to add additional advantageous properties to the prepresent fiber properties that contributed to the fact that almost 70% of the apparel fibers used in the United States in 1952 were cotton fibers. In accordance with this invention, these particularly valuable fibers can be produced by: etherifying cotton fibers by reacting such fibers in the presence of aqueous alkali metal hydroxide with an etherifying agent selected from the group consisting of 2-aminoethyl sulfure acid, monochloroacetic acid, ethylene oxide, acrylonitrile, and dimethyl sulfate, to produce cotton fibers containing from about 0.1 to 1.0 of the etherifying radicals of the etherifying agent per anhydroglucose unit; and reacting the etherified fibers with beta-propiolactone by impregnating them with an aqueous liquid, which may be water or water containing aqueous alkali metal hydroxide, immersing the impregnated fibers in a solution of beta-propiolactone in an unreactive liquid solvent containing from about 5 to 95 parts of beta-propiolactone per part of solution, and maintaining the solution at from about 5 to 50° C. until the fibers contain from about 10 to 20%, based on the weight of the etherified fibers, of beta-propiolactone reaction products combined with cellulose.

The chemically modified cellulosic fibers produced by this invention are useful for substantially any of the wide variety of uses known for cellulosic fibers. Those containing less than about one polar alkyl radical per anhydroglucose unit are particularly useful as textile fibers wherever wool-like properties and properties such as a heat resistance, an acid induced degradation resistance and a wrinkle resistance markedly greater than those of cotton fibers is important.

The fibers produced by this invention can readily be produced in the form of unsaturated compositions which undergo the reactions typical of organic compounds containing olefinic groups. These unsaturated fibers constitute valuable intermediates from which to prepare numerous different derivatives of cellulose in the form of cotton fibers.

The unsaturated fibers can be produced by subjecting the fibers produced by etherification and beta-propiolactone reaction to dehydration at moderately elevated temperatures. A preferred process of producing them, comprises, immersing such fibers in a water immiscible inert organic liquid, refluxing the liquid, and isolating water from the liquid returning from the condenser. The water immiscible solvents for beta-propiolactone are preferred liquids for such employment. The dehydration is preferably conducted at from about 50° C. to about 150° C. The dehydration can be conducted by a wide variety of conventional procedures for dehydrating solid compositions at moderately elevated temperatures. It can be conducted during the reaction of the etherified cellulose fiber with beta-propiolactone, so that the beta-propiolactone reacted fibers are subjected to dehydration as they are formed.

The following examples further illustrate this invention.

#### EXAMPLE 1

Weighed samples of the following forms of cotton fibers were each reacted with beta-propiolactone. The samples were each immersed in about 20 times their weight of a xylene solution of beta-propiolactone containing about 10% by weight of propiolactone. The solutions containing the immersed samples were refluxed

under atmospheric pressure for about one hour. Each sample of the so-treated fibers was extracted for about 60 minutes with acetone, to remove reactants and byproducts, then dried and weighed. The amount by which the weight of the samples was increased by the treatment is reported as percent weight gain in the following table.

The samples used were: (a) A skein of plain cotton thread, purified by extraction with monoethanolamine; (b) a skein of mercerized cotton thread; (c) a piece of hydroxyethylated cotton cloth containing 9.25%  $C_2H_4O$  (prepared by reacting sodium-hydroxide-treated cloth with a 1.6% solution of ethylene oxide in carbon tetrachloride for 1 hour at 55° C.); (d) a skein of cyanoethylated cotton thread containing 2.3% N (prepared by reacting sodium-hydroxide-treated thread with acrylonitrile at 55° C.); (e) a piece of aminoethylated cotton cloth containing 0.88% N (prepared by padding cotton cloth with a solution of 20% 2-aminoethyl sulfuric acid in 40% sodium hydroxide solution and heating at 110° C. for 30 minutes); (f) a skein of carboxymethylated cotton thread containing 0.07 sodium carboxymethyl groups per anhydroglucose unit (prepared by padding cotton thread with 15% monochloroacetic acid followed by treatment with 40% sodium hydroxide); and (g) a skein of partially methylated cotton thread containing 7.8%  $OCH_3$  (prepared by reacting sodium hydroxide-treated cotton thread with methyl sulfate in toluene).

Table of results

| Material                 | Weight gain percent | 30 |
|--------------------------|---------------------|----|
| Purified cotton          | 29.6                |    |
| Mercerized cotton        | 24.5                |    |
| Hydroxyethylated cotton  | 77.0                |    |
| Cyanoethylated cotton    | 55.2                |    |
| Aminoethylated cotton    | 88.5                | 35 |
| Carboxymethylated cotton | 57.9                |    |
| Methylated cotton        | 38.8                |    |

EXAMPLE 2

Samples of cotton cloths which had been hydroxyethylated, aminoethylated, and carboxymethylated in the manner described in Example 1, and a sample of plain cotton cloth, were padded to 131-146% wet pickup of 10% sodium hydroxide solution and then soaked in a 20% aqueous solution of beta-propiolactone for 1 hour at normal room temperature. After the treatment, the samples were extracted with boiling water to remove reactants and by-products, dried and weighed.

Table of results

| Material                                  | Wet pickup of NaOH% | Weight gain, percent | 55 |
|-------------------------------------------|---------------------|----------------------|----|
| Hydroxyethyl cellulose (9.25% $C_2H_4O$ ) | 143                 | 23.4                 |    |
| Aminoethyl cellulose (0.43% N)            | 139                 | 19.8                 |    |
| Carboxymethylcellulose (D.S.: 0.08)       | 146                 | 22.9                 |    |
| Plain cotton                              | 131                 | 8.7                  |    |

EXAMPLE 3

A piece of plain cotton cloth and a piece of aminoethylated cotton cloth (containing 0.88% N, and prepared as described in Example 1) were treated with pure beta-propiolactone at room temperature for 1 hour. After extraction and drying, neither sample had gained weight.

However, when pieces of the same cloths were padded with water to about 100% wet pickup, then soaked in pure beta-propiolactone for 1 hour; the weight gain of the plain cotton was 1.9%, and that of the aminoethylated cotton cloth was 8.6%.

And, when pieces of the same cloths were similarly padded with 10% sodium hydroxide prior to soaking in beta-propiolactone, the weight gain of the plain cotton cloth was 16.5%, and that of the aminoethylated cotton cloth was 24.7%.

When a piece of the same aminoethylated cotton cloth was padded to 59.4% wet pickup of water and then treated with excess pure beta-propiolactone at about 95°-99° C. for 1 hour; the weight gain was 149.8%.

## EXAMPLE 4

Skeins of partially carboxymethylated cotton 7/2 thread containing 0.07 sodium carboxymethyl groups per anhydroglucose unit (prepared as described in Example 1) were treated with 20 times their weight of 10% beta-propiolactone in xylene at reflux temperature for various periods of time (1-60 min.). Weight gains shown in the table below indicate that the reaction (with the conditions used) was essentially complete after 20 minutes.

The thread before lactone-treatment was somewhat stiff, but was considerably softened after reaction with beta-propiolactone. This softening effect increases as the amount of beta-propiolactone substituents increases. When warm, the treated thread was much softer than it was at room temperature. This effect is possibly due to the thermoplastic properties of the beta-propiolactone substituents.

| Reaction time (min.) | Wt. gain (percent) | Reaction time (min.) | Wt. gain (percent) |
|----------------------|--------------------|----------------------|--------------------|
| 1                    | 4.4                | 20                   | 58.6               |
| 5                    | 16.3               | 40                   | 60.5               |
| 10                   | 35.7               | 60                   | 57.9               |

EXAMPLE 5

Skeins of partially carboxymethylated cotton 7/2 thread similar to those used in Example 4 were treated with 20 times their weight of various concentrations of beta-propiolactone in xylene, at reflux, for 1 hour. Results are shown in the table below.

| Conc. of BPL (percent): | Weight gain (percent) |
|-------------------------|-----------------------|
| 0 (control)             |                       |
| 5                       | 29.6                  |
| 10                      | 51.2                  |
| 15                      | 84.0                  |
| 20                      | 122.3                 |

EXAMPLE 6

Partially carboxymethylated cotton cloth containing 0.06 carboxymethyl groups per anhydroglucose unit (prepared as described in Example 1) in the acid form, and as the sodium salt, along with a mercerized cotton cloth and a plain cotton cloth were treated with a xylene solution containing beta-propiolactone in an amount providing twice the weight of the cloth of beta-propiolactone, at reflux for 30 minutes. Weight gains after extraction with acetone are shown in the table below.

| Cloth:                                | Wt. gain (percent) |
|---------------------------------------|--------------------|
| Plain cotton                          | 29.8               |
| Mercerized cotton                     | 16.8               |
| Carboxymethylated cotton, acid form   | 11.3               |
| Carboxymethylated cotton, sodium salt | 181.5              |

EXAMPLE 7

Plain 12/5 sewing thread and carboxymethylated 12/5 thread containing 0.08 carboxymethyl groups per anhydroglucose unit (prepared as described in Example 1) in the form of the free acid and the sodium salt, were treated with beta-propiolactone to about 12% weight gain (after extraction with acetone to remove unattached polymer). The treated samples and an untreated sample of the etherified cotton thread were then extracted ten times with hot glacial acetic acid. The treated plain cotton retained 50% of its original tensile strength while the sodium salt of the treated etherified cotton retained 90% and the free acid form of the treated etherified cotton retained 85%. The untreated etherified cotton thread retained 65%. This showed that carboxymethylation and beta-propiolactone reaction coact to give enhanced protection against acetic acid degradation.

## EXAMPLE 8

A duplicate set of the samples used in Example 7 were exposed to  $\text{NO}_2$  gas in a closed desiccator for 6 hours. The treated plain cotton retained 70% of its tensile strength while the treated acid etherified sample retained 100% and the treated sodium etherified sample retained 90%. The untreated etherified sample retained 52%.

## EXAMPLE 9

When part of the above samples were heated at 125° C. for 15 days, the strength retention of the treated etherified cotton was approximately 10-15% better than that of either the treated plain cotton or the untreated etherified cotton.

We claim:

1. A process comprising etherifying cellulose fibers with an etherifying agent selected from the group consisting of aminoalkyl sulfuric acid, monochloroacetic acid, alkylene oxide, acrylonitrile, and alkyl sulfate, until esterified cellulose fibers containing from about 0.1 to 2.5 of the etherifying radicals of said etherifying agent per anhydroglucose unit are produced, the alkyl group in each of said etherifying radicals having from 1 to 3 carbon atoms, and reacting the said etherified cellulose fibers with beta-propiolactone at a temperature of from about 0° C. to a temperature slightly below the decomposition temperature of the fibers until fibers are produced containing from about 0.5 to 26%, based on the weight of the etherified fibers, of beta-propiolactone reaction products combined with the cellulose.
2. The process of claim 1 wherein the etherifying agent is aminoalkyl sulfuric acid.
3. The process of claim 2 wherein the aminoalkyl sulfuric acid is 2-aminoethyl sulfuric acid.

4. The process of claim 1 wherein the etherifying agent is monochloroacetic acid.

5. A process comprising etherifying cotton fibers by reacting said fibers in the presence of aqueous alkali metal hydroxide with an etherifying agent selected from the group consisting of aminoalkyl sulfuric acid, monochloroacetic acid, alkylene oxide, acrylonitrile, and alkyl sulfate until etherified cotton fibers containing from about 0.1 to 1.0 of the etherifying radicals of said etherifying agent per anhydroglucose unit are produced, the alkyl group in each of said etherifying radicals having from 1 to 3 carbon atoms, and reacting the said etherified cotton fibers with beta-propiolactone by impregnating them with water to improve their reactivity towards beta-propiolactone, immersing the so-impregnated etherified cotton fibers in a solution of beta-propiolactone in an unreactive liquid solvent containing from about 5 to 95 parts of beta-propiolactone per part of solution, and maintaining the solution at from about 5° to 50° C. until the fibers contain from about 10 to 20%, based on the weight of the original etherified fibers, of beta-propiolactone reaction products combined with the cellulose.

6. The process of claim 5 wherein the water, with which the etherified fibers are impregnated to improve their reactivity toward beta-propiolactone, also contains from about 5 to 50% alkali metal hydroxide to further improve said reactivity of the etherified fibers towards beta-propiolactone.

7. The process of claim 5 wherein the etherifying agent is 2-aminoethyl sulfuric acid.

8. The process of claim 5 wherein the etherifying agent is monochloroacetic acid.

No references cited.